

## UNITED STATES PATENT OFFICE

1,963,239

## GEAR LUBRICANT

George M. Maverick, Elizabeth, N. J., assignor to  
Standard Oil Development Company

No Drawing. Application April 15, 1931,  
Serial No. 530,433

2 Claims. (Cl. 87—9)

This invention relates to heavy lubricants and a method for preparing them. More particularly it relates to gear oils such as those used for lubricating transmission gears, differential gears and other similar mechanisms which require a heavy lubricant that must remain fluid and plastic at relatively low temperatures, and in one phase the invention relates to a gear oil containing a specific depressant of channeling, as will be more fully hereinafter described.

I have discovered that by incorporating these heavy lubricants with certain unctuous synthetics, for example heavy condensation products of paraffinic and aromatic hydrocarbons, the plasticity and fluidity of the lubricants at low temperatures is markedly greater than that of the normal heavy lubricant. The method of preparing the modified lubricants and the nature of the unctuous synthetics will be fully understood from the following description.

The term unctuous synthetic as used here and in the claims will be understood to mean a heavy hydrocarbon condensation product prepared from hydrocarbons having a molecular weight of at least 170 and containing at least 13.5 to 15 parts of hydrogen for each 100 parts of carbon, the hydrogen content being the higher the lower the molecular weight. Open-chain hydrocarbons, such as the paraffins are preferable as starting materials for the preparation of these synthetics, and especially valuable products are obtained by condensing the open-chain hydrocarbons in the presence of cyclic or olefinic hydrocarbons. The unctuous synthetics are characterized by high viscosity indices, generally over 100, high flash points, generally over 500° F., and high Saybolt viscosities at 100° F., generally over 1000, and ranging as high as 2000, 5000, 10,000 or 20,000 seconds or more. They also have high molecular weights and are in general very viscous. The methods by which they may be prepared will be described below.

The modified lubricants may be prepared as follows. A heavy hydrocarbon oil with Saybolt viscosity at 210° F. between say 100 and 200 seconds or higher is heated to a temperature of about 150 to 180° F. and from 2 to 10% or more by weight of unctuous synthetic is added. On cooling, the modified oil remains homogeneous and the unctuous synthetic does not show any tendency to separate out. It is preferable to add about 2 to 5% of the unctuous synthetic, but larger amounts, say 10 to 20% or more may be added. In general, however, the maximum beneficial effect is obtained with about 2 to 3%. In

some gear oils not subject to extreme service conditions it may be feasible to use less than 2% of the unctuous synthetic, the proportion ranging as required downwardly even to a fraction of 1%.

The modified lubricants have greater plasticity and fluidity at low temperatures than the unmodified oils, and for this reason the gear shifting effort, drag resistance and tendency to channel when the modified lubricants are cold, as in starting, are greatly reduced. In cold weather particularly, or where the oils are used in low temperature work, the increased plasticity and fluidity at low temperatures of the modified oils is of great advantage. It makes the handling and pumping of the lubricant easier, it reduces the power loss due to friction of the moving parts, it results in less wear and abrasion on the gears, and reduces the operating temperature in the gear housings. Moreover, the tendency of ordinary gear lubricants to channel, that is to become so viscous that the gears cut channels in the oily mass instead of spinning in continuous contact with fluid oil, is very marked at low temperatures. By the addition of small amounts of the unctuous synthetic the channeling temperature is lowered from 10 to 15° F. or more.

It should be particularly noted that only small amounts of the unctuous synthetic are required to serve effectively as an anti-channelant or depressant of channeling, as the effect may be termed. This, of course, is a very different result from that obtainable by adding an ordinary thinner or thinning oil such as kerosene. The unctuous synthetic cannot, of course, be classed as a diluent of this type since it does not reduce the lubricating qualities of the oil as in itself the unctuous synthetic preferably is produced of a character exhibiting excellent lubricating values. Looking at the modified lubricant from one standpoint it may be regarded as containing a wax protective colloid capable of substantially reducing the critical temperature of congelation.

In the case of compounded oils, where 2, 5, 7, 10% or more of metallic soaps, such as lead, sodium or aluminum oleates or stearates is added to the straight base mineral oil, the solubility of the soaps in the oil is not very great. It is essential, however, to keep them in solution to prevent them settling out and caking on the moving parts causing undue abrasion and wear. Incorporating unctuous synthetic with such compounded oils appears to aid in retaining these soaps in solution, as little as about 2% of the unctuous synthetic being effective for this purpose. In some cases, the addition of the unctuous

synthetic also decreases the foaming of the oil on agitation.

The synthetic to be added to the heavy lubricating oil may be prepared in a variety of different ways and from a number of different materials.

- One type of unctuous synthetic is prepared by condensing naphthalene on chlorinated paraffin in the presence of  $AlCl_3$ . The paraffin wax is chlorinated by direct addition of chlorine until about 10-15% by weight of chlorine has been added. The chlorination is preferably carried out above the melting point of the paraffin but below the decomposition temperature of the chlorparaffin, say between about 180 and 300° F. and iodine crystals or sunlight, or both may be used to catalyze the chlorination. The chlorparaffin is then dissolved in a highly saturated hydrocarbon oil preferably of the kerosene range and naphthalene is added to this solution. About 20 parts by weight of naphthalene to about 100 parts of chlorparaffin is a satisfactory proportion. The resulting solution is then agitated thoroughly by mechanical or other stirring means and heated to a temperature between about 60° and 175° F., between 100 and 110° F. being preferable. While agitated at this temperature anhydrous aluminum chloride is slowly added over a period of from 4 to 6 hours, until about 7 to 8 parts by weight have been added in all. The reaction is allowed to continue then for from 4 to 24 hours longer. It is preferable to allow the reaction to proceed without the application of heat or refrigeration.

When the reaction is complete, the sludge is separated from the oil by settling, centrifuging, or other means. The clear oil is then treated with concentrated sulfuric acid and clay. After removing the clay the oil is distilled either by fire and steam or by vacuum distillation. The distillate comprises the light mineral oil solvent used, some light lubricating oil and a small amount of unconverted wax. The residue is the desired unctuous synthetic. The following is a typical inspection of a synthetic prepared in this way:

- Gravity A. P. I. 22.1°  
 Saybolt viscosity @ 100° F. 4777 sec.  
 Saybolt viscosity @ 210° F. 269 sec.  
 Viscosity index 110  
 Flash 580° F.  
 Carbon 1.08%  
 Color, Robinson 5 1/2  
 Chlorine 0.031%

It will be understood that the proportions of materials used and the conditions of treatment may be varied considerably with equally satisfactory results, and that the resultant unctuous synthetic may vary therefore to some extent in characteristics. Unconverted wax, recovered solvent, and wax obtained from the sludge may be returned to the process.

An unctuous synthetic may be prepared from chlorinated paraffin and benzol by substantially the same method. An inspection of such an oil follows:

- Gravity A. P. I. 25.8°  
 Saybolt viscosity @ 100° F. 1743 sec.  
 Saybolt viscosity @ 210° F. 134 sec.  
 Viscosity index 108  
 Flash 550° F.  
 Carbon 0.679%  
 Color, Robinson 4 1/2  
 Chlorine 0.031%

75 An unctuous synthetic prepared from chlo-

minated paraffin and an aromatic gas oil fraction has the following inspection:

|                             |           |
|-----------------------------|-----------|
| Gravity A. P. I.            | 21.7      |
| Saybolt viscosity @ 100° F. | 5200 sec. |
| Saybolt viscosity @ 210° F. | 268 sec.  |
| Flash                       | 565° F.   |
| Carbon                      | 3.054%    |

Another type of unctuous synthetic may be prepared without the use of aromatic compounds. This is made by condensing a cracked chlorinated paraffin in the presence of aluminum chloride. Crude scale wax is chlorinated to about 10 to 25% by weight chlorine, and is then passed through a heating coil at a temperature of about 600 to 750° F. preferably in the presence of a catalytic material such as  $BaCl_2$ . At the high temperature, hydrogen chloride is split off, leaving an unsaturated product with only about 3% chlorine content. This unsaturated product is then diluted with a light mineral oil solvent and is condensed in the presence of aluminum chloride. The kind of unctuous synthetic obtained depends upon the chlorine content of the chlorinated paraffin. Inspections of synethetics obtained from chlorinated paraffin containing 10 and 25% of chlorine by weight follow:

|                             | Chlorparaffin containing 25% $Cl_2$ | Chlorparaffin containing 10% $Cl_2$ | 105 |
|-----------------------------|-------------------------------------|-------------------------------------|-----|
| Gravity A. P. I.            | 26.4                                | 29.8                                |     |
| Saybolt viscosity @ 100° F. | 1630 sec.                           | 3000 sec.                           |     |
| Saybolt viscosity @ 210° F. | 167 sec.                            | 234 sec.                            |     |
| Viscosity index             | 128                                 | 117                                 |     |
| Flash                       | 485° F.                             | 620° F.                             | 110 |
| Carbon                      | 1.53%                               | 1.06%                               |     |
| Pour                        | 70° F.                              | 80° F.                              |     |

Still another type of unctuous synthetic may be prepared by condensing a chlorinated fatty acid such as stearic acid with benzol, naphthalene or other aromatic compounds in the presence of aluminum chloride.

The following examples will illustrate the effect of adding small amounts of unctuous synthetics to heavy lubricants.

A straight transmission oil is run in a Chevrolet transmission, first without any synthetic added and then with 2% unctuous synthetic added. The results are as follows:

|                                                                                                        | Straight transmission oil | With 2% unctuous synthetic |     |
|--------------------------------------------------------------------------------------------------------|---------------------------|----------------------------|-----|
| Gear shift effort                                                                                      | 307 lbs. secs.            | 189 lbs. secs.             | 130 |
| Starting drag                                                                                          | 26 lbs.                   | 20 lbs.                    |     |
| Drag resistance to spin dynamometer at 60 R. P. M.                                                     | 49 1/2 lbs.               | 37 1/2 lbs.                |     |
| The results of other tests on the two oils are as follows:                                             |                           |                            |     |
| Temperature at which channeling occurs                                                                 | 12° F.                    | 2° F.                      |     |
| Penetration test at -13° F. Time for steel bar 9 1/4" long, 3/4" diameter to penetrate 1 inch into oil | 74 secs.                  | 19 secs.                   | 135 |
| Penetration test at -33 1/2° F. Time for bar to penetrate 1/8 of an inch                               | 200 secs.                 | 95 secs.                   |     |

The penetration test at -14° F. on a compounded oil containing 10% lead oleate showed that 35 seconds was required for the bar to penetrate 1 inch. When 2% unctuous synthetic was added to this oil only 42 seconds were required for the same bar to penetrate 1 inch.

These tests uniformly show that the addition of small percentages of unctuous synthetic of the nature described above to heavy lubricants materially increases the fluidity and plasticity of such lubricants at low temperature.

Although the beneficial effect of the addition of the unctuous synthetic is most noticeable at low temperatures, it should be understood that the presence of the unctuous synthetic in no way 5 impairs the effectiveness of the lubricant at normal operating temperatures. The following comparison of the inspection of a transmission oil before and after the addition of 2% unctuous synthetic shows how little the synthetic affects 10 the normal characteristics of the lubricant:

characterized by high pour points and the addition of unctuous synthetics to such lubricants may therefore be of particular advantage.

The term "gear oil" is used in the following 80 claims to designate a heavy fluid or plastic lubricant with a Saybolt viscosity above about 100 seconds at 210° F.

This invention is not limited by any theory of the mechanism of the effect of unctuous synthetics on heavy lubricants nor by any details given merely by way of illustration, but is limited only by the following claims in which I wish to claim all novelty inherent in the invention. 85

I claim:

1. Lubricant composition comprising a gear oil 90 incorporated with a few per cent. of an unctuous synthetic depressant of channeling comprising a hydrocarbon condensation product having an initial molecular weight of at least 170 and containing at least 13.5 parts of hydrogen per 100 parts of carbon and a metallic soap soluble in said composition.

2. Composition according to claim 1 containing not more than about 10% of a metallic soap of a fatty acid. 95

100  
GEORGE M. MAVERICK.

|                             | Straight transmission oil | Plus 2% unctuous synthetic |
|-----------------------------|---------------------------|----------------------------|
| 15 Gravity, A. P. L.        | 20.9                      | 20.9                       |
| Saybolt viscosity @ 100° F. | 1988                      | 1980                       |
| Saybolt viscosity @ 210° F. | 112                       | 114                        |
| Pour                        | 15                        | 16                         |

20 The unctuous synthetics may also be added in small quantities to heavy hydrogenated lubricants, that is heavy oils with Saybolt viscosity at 210° F. above about 100 obtained by the hydrogenation of heavy residues, topped crudes, heavy 25 lubricating distillates and similar heavy fractions. The hydrogenated oils are in general

30 characterized by high pour points and the addition of unctuous synthetics to such lubricants may therefore be of particular advantage. 105

35 The unctuous synthetics may also be added in small quantities to heavy hydrogenated lubricants, that is heavy oils with Saybolt viscosity at 210° F. above about 100 obtained by the hydrogenation of heavy residues, topped crudes, heavy 40 lubricating distillates and similar heavy fractions. The hydrogenated oils are in general

45 characterized by high pour points and the addition of unctuous synthetics to such lubricants may therefore be of particular advantage. 110

50 The unctuous synthetics may also be added in small quantities to heavy hydrogenated lubricants, that is heavy oils with Saybolt viscosity at 210° F. above about 100 obtained by the hydrogenation of heavy residues, topped crudes, heavy 55 lubricating distillates and similar heavy fractions. The hydrogenated oils are in general

60 characterized by high pour points and the addition of unctuous synthetics to such lubricants may therefore be of particular advantage. 115

65 The unctuous synthetics may also be added in small quantities to heavy hydrogenated lubricants, that is heavy oils with Saybolt viscosity at 210° F. above about 100 obtained by the hydrogenation of heavy residues, topped crudes, heavy 70 lubricating distillates and similar heavy fractions. The hydrogenated oils are in general

75 characterized by high pour points and the addition of unctuous synthetics to such lubricants may therefore be of particular advantage. 120

80 The unctuous synthetics may also be added in small quantities to heavy hydrogenated lubricants, that is heavy oils with Saybolt viscosity at 210° F. above about 100 obtained by the hydrogenation of heavy residues, topped crudes, heavy 85 lubricating distillates and similar heavy fractions. The hydrogenated oils are in general

90 characterized by high pour points and the addition of unctuous synthetics to such lubricants may therefore be of particular advantage. 125

95 The unctuous synthetics may also be added in small quantities to heavy hydrogenated lubricants, that is heavy oils with Saybolt viscosity at 210° F. above about 100 obtained by the hydrogenation of heavy residues, topped crudes, heavy 100 lubricating distillates and similar heavy fractions. The hydrogenated oils are in general

105 characterized by high pour points and the addition of unctuous synthetics to such lubricants may therefore be of particular advantage. 130

110 characterized by high pour points and the addition of unctuous synthetics to such lubricants may therefore be of particular advantage. 135